

Nov. 29, 1938.

A. H. WARTH

2,138,439

CONTAINER CLOSURE AND LINING MATERIAL THEREFOR

Filed March 31, 1936

*Fig. 1.*



*Fig. 3.*



*Fig. 2.*



*Fig. 4.*



Inventor

*Albin H. WARTH*

By *Lehman, Dwyer & Lehman*  
Attorneys

## UNITED STATES PATENT OFFICE

2,138,439

CONTAINER CLOSURE AND LINING  
MATERIAL THEREFOR

Albin H. Warth, Baltimore, Md., assignor to  
Crown Cork & Seal Company, Inc., Baltimore,  
Md., a corporation of New York

Application March 31, 1936, Serial No. 71,917

2 Claims. (Cl. 215—39)

The present invention relates to container closures and particularly to closures of the center spot crown type. Caps of this type comprise a metallic shell having a crimped skirt, a cushion liner of natural cork or cork composition, and a facing layer of smaller diameter than the cushion disc, adhesively secured to the disc to cover the central portion thereof, and to leave exposed an annular marginal portion, adapted to 5 cooperate with the exterior portion of the sealing lip of the bottle neck to provide a tight seal. As is well known, the center spot constitutes a liner and prevents the contents of the bottle from coming in contact with the cushion disc.

15 In the past, satisfactory results have been obtained by using metal foils, such as aluminum foil, as the lining material. Such foils have been adhesively united to the cushion disc by means of thermoplastic adhesives, so that the caps and 20 spots can be rapidly assembled by uniting the spots to the cushion discs by heat and pressure.

Attempts have been made to use exteriorly varnished paper as a spotting material, and fairly 25 satisfactory results have been accomplished by combining a sheet of paper, having a varnish coat on its exterior surface, with an interior layer of gutta percha, the latter acting as a thermoplastic adhesive between the paper face of the spot and the cork cushion. However, 30 certain defects have been encountered in the commercial use of such single surface varnished spots. For instance, the capillarity of the paper inwardly of the varnish layer results in absorption of the liquid contents of the bottle by 35 the paper, particularly in connection with the sealing of beverages which must be subjected to a pasteurizing or sterilizing operation, such as beer. Any minute break in such a varnish coating results in permitting the liquid to penetrate 40 the spot and soften the paper. If paper of the bleached kraft type is used, the spot will be subjected to an undesirable swelling action and disintegration which renders the spot useless and causes the beverage to deteriorate in quality.

45 The same difficulty is encountered with other papers such as Express paper, although to a lesser degree.

Attempts have been made to avoid this capillary absorption of the paper by saturating the 50 paper with varnish, or coating it on both surfaces, but a satisfactory spot of this type could not be made, prior to the present invention, because the gutta percha adhesive would not adhere with sufficient tenacity to a varnished surface. Consequently, when a sheet of kraft paper

or the like was given a coating of varnish on its inner and outer surfaces, it could not be satisfactorily adhesively united to the cork cushion by the standard thermoplastic adhesive of the prior art, i. e., gutta percha. As a result, all 5 commercial varnish paper spots, prior to the present invention, consisted of a layer of paper, a single outer layer of varnish, and an inner layer of gutta percha united directly to the inner, uncoated paper face of the spot, and even so, 10 the paper spots were not as commercially satisfactory as the metal foil spots.

In my prior United States Patent No. 1,956,481, April 24, 1934, I have disclosed and claimed a novel spot for crown caps, comprising a metal 15 foil disc, or a single surface varnished paper disc, in combination with a novel thermoplastic adhesive comprising a nitrocellulose and a resin. When used with metal foil, this adhesive has been found to be far superior to gutta percha. 20 It has gone into wide commercial use as a means for uniting foil spots to the cushion liners of crown caps.

When attempts were made to substitute this new adhesive material for gutta percha, as a 25 means for securing varnish coated paper spots of the prior art to the cushion liners of crown caps, somewhat unsatisfactory results were encountered. I discovered that, in order to make a 30 satisfactory bond, the nitrocellulose-resin adhesive must be in the form of a continuous surface layer or film on the material, such as paper or foil, with which it is to be used. If it is absorbed by the web of material, the surface layer will be discontinuous and will lack the 35 continuity of a film. At the places where such absorption occurs and where the film is broken, the adhesive effect under heat and pressure is poor. When attempts were made to use such an adhesive with the single surface varnish coated 40 papers of commercial type, as a substitute for the more expensive gutta percha adhesive, I discovered that the absorption of the adhesive by the paper was such as to destroy the uniform 45 filming of the adhesive and resulted in a poor bond between the paper and the cushion layer. Consequently, prior to the present invention, it was thought that the recently developed nitrocellulose-resin could not displace gutta percha adhesives in the varnished paper spot art, and 50 that it would be useful only in connection with metallic foil spotting materials.

Upon discovering the cause of the defect in the action of the nitrocellulose-resin type of thermoplastic adhesive when used with paper 55

spots, namely, the absorption of the adhesive by the paper, I conceived the idea of preventing the absorption by first coating both faces, instead of the outer face only, with an appropriate 5 varnish solution. As stated above, the former attempts to use a paper spot having both faces coated with varnish were unsuccessful because a satisfactory thermoplastic adhesive was not then known. I discovered, however, that the 10 recently developed nitrocellulose-resin adhesive resulted in a highly satisfactory bond between an interior varnish coat on a paper spot and the cork liner. Moreover, absorption of the adhesive into the paper was thereby prevented, and a spot 15 of high efficiency produced.

Thus, the combination of the present invention results in gaining all of the advantages of a double coated varnish paper spot, together with all of the advantages of the nitrocellulose-resin 20 adhesives. The two coatings of varnish on the paper saturate the paper fibres to such an extent that absorption of the contents of the bottle by the paper is effectively prevented, and the capillarity of the paper eliminated. The nitro- 25 cellulose-resin adhesive films out upon the inner varnish layer of the paper spot with the desired continuity, and the spot so coated with an inner layer of a varnish cooperates with the nitrocellulose-resin adhesive with the same efficiency 30 as a metal foil spot.

The present invention is not limited to the use of a thermoplastic adhesive of the type disclosed in my prior Patent No. 1,956,481, referred to above, as I have found that other thermoplastic 35 adhesives may be used to form a suitable bond between the cork cushion and the inner varnish face of a paper spot. Such adhesives include chlorinated rubber-resin adhesives, and an adhesive comprising an ethyl ester of shellac and 40 nitrocellulose.

The varnish coating used on the inner and outer faces of the paper spot may be either an oil varnish solution, or a synthetic resin varnish.

Although the paper preferred is a bleached 45 kraft paper, because of its strength and cheapness, the invention is not confined to its use, as any good strong paper may be substituted. Express paper, for certain types of spots, has been found to be particularly satisfactory.

50 A typical oil varnish for coating the paper may be made in accordance with the following formula:

|                                            |  |
|--------------------------------------------|--|
| 100 pounds oil soluble 100% phenolic resin |  |
| 55 27 gallons China-wood oil               |  |
| 3 gallons four hour bodied linseed oil     |  |
| 72 ounces cobalt drier                     |  |
| 63 ounces manganese drier                  |  |
| 65 gallons mineral spirits                 |  |

60 **Cook.**—The resin and China-wood oil are heated together to 470° F. in about thirty-four minutes. Hold for body and get three and one-half foot string on piece of metal. Add bodied linseed oil and cool to 440° F. Add mineral spirits 65 and dryers.

A typical synthetic resin varnish for coating or saturating the paper may be made in accordance with the following formula:

|                                        |       |
|----------------------------------------|-------|
| 70 Synthetic resin (e. g. rezyl resin) | Parts |
| Butyl acetate                          | 20    |
| Ethyl acetate                          | 20    |
| Butyl cellosolve                       | 20    |

75 The oil varnish is characterized by its high

viscosity, the use of high boiling solvents, the limited penetration into the paper, and the requirement for thorough baking or drying of the coating to polymerize and oxidize the oil containing constituent.

The synthetic resin solution varnish is of lower viscosity, and its solvents are a mixture of lower and higher boiling solvents. It penetrates the paper quite rapidly, and the drying may be accomplished in a short time cycle.

It should be understood that the organic solvents for the resin solution varnishes are not limited to those given in the above formula, as such solvents as cellosolve (B. P. 135° C.), methyl n. amyl ketone (B. P. 147°-152° C.), 15 hexone (B. P. 113-119° C.), acetone (B. P. 56° C.), methyl acetone (B. P. 50-67° C.), and toluol (B. P. 110° C.) are all useful for such resin solutions.

The thickness of the paper layer is selected according to the factors of (1) the degree of penetration, (2) its physical strength, and (3) its cost. For coating with oil varnishes, the paper is preferably within the range of .0035" to .0045". For dip resin solutions it should be between .0025" and .0035". The varnish films bring these papers in coated condition to a greater thickness, e. g., .0053" for a .0045" paper, and .0042" for dipped .0035" paper. The nitrocellulose-resin adhesive film is .0015" to .0025" thick. 30 The invention, of course, is not to be confined to these particular thicknesses of paper, varnish, and/or adhesive. It is usually desirable to keep the finished coated paper thickness below .006". To this the thickness of the adhesive should be 35 added.

Several different methods may be employed to apply the varnish coatings on the two surfaces of the paper. For instance, the paper may be passed through a dip tank and the excess varnish removed by felt wipers or the like. Such a process is preferred where the thinner varnishes are used, such as synthetic resin varnishes, and if the solution is sufficiently thin, no wipers are needed. If the varnish is somewhat viscous, it can be applied satisfactorily with coating rolls, for instance, by the use of a fountain with pick-up distributor and applicator rolls for one side, and a similar set for the other side. Drying may be accomplished in a vertical oven 50 in which the varnish coated paper is festooned by running the same over supporting rolls at the top of the oven, and then down for rewind. The oil varnish described above should be dried at 220° F. for twenty-five minutes. The resin solution may be dried at 260° F. for ten to twelve minutes as will be appreciated, such varnishes are not thermo-plastic.

In the accompanying drawing:

Figure 1 shows an enlarged plan view of a spot 60 crown according to the present invention.

Figure 2 is a vertical sectional view, on an enlarged scale, of the device of Figure 1.

Figure 3 is a diagrammatic plan view of the spot of the present invention, with the various 65 layers exposed to view.

Figure 4 is a greatly enlarged cross sectional view of the laminated material which is used to form the spot of the present invention.

In the drawing, a crown cap is shown comprising a metallic shell 10 having the usual top 70 11 and a down-turned crimped skirt 12. A cushion liner 13 which may be either natural cork or a granulated cork composition, is adhesively united to the interior of the shell by an appro- 75

priate adhesive 14. The center spot 15 is secured concentrically to the inner face of the cushion liner 13. The spot comprises a layer of paper 16, an outer varnish layer 17, an inner varnish layer 18, and a thermoplastic adhesive layer 19. The spot is preferably secured to the cushion disc by heat and pressure.

The paper layer 16 preferably is a smooth finished, bleached kraft paper, although other papers, such as Express, are satisfactory.

The varnish layers 17 and 18 may consist of either an oil varnish, or a resin varnish, of the types discussed above. Preferably, the varnish penetrates the paper somewhat, as indicated diagrammatically in Figure 4, and the capillarity of the paper and, consequently, its tendency to absorb the contents of the bottle, is thus diminished. As a result, an impervious facing 17 is presented to the contents of the bottle, and an impervious surface 18 is provided upon which the adhesive may be spread in a continuous film, without any penetration into the paper.

The thermoplastic adhesive 19 may be of the type described in detail in my prior Patent No. 2,1956,481, or it may comprise a chlorinated rubber-resin adhesive. An adhesive of a suitable type may comprise 20 parts 50% solution of ethyl ester of shellac and 15 parts of 10% solu-

tion of nitrocellulose (5 sec.) Such an adhesive has been found to be particularly efficient as a bonding medium between an inner varnished surface of a paper spot and a cork disc.

I claim:—

1. In a cap which includes a metal shell and a cushion liner, a facing of the center spot type of lesser diameter than the cushion liner, said facing comprising a layer of paper having a non-thermoplastic varnish coating on both its faces and a continuous layer of thermoplastic adhesive comprising a cellulose ester and a resin between its inner varnished face and said cushion liner, said varnish rendering the paper non-adsorptive to and being adhesively compatible with said adhesive. 10

2. In a cap which includes a metal shell and a cushion liner, a facing of the center spot type of lesser diameter than the cushion liner, said facing comprising a layer of paper having a non-thermoplastic varnish coating on both its faces and a continuous layer of thermoplastic adhesive comprising nitro-cellulose and a resin between its inner varnished face and said cushion liner, said varnish rendering the paper non-adsorptive 20 to and being adhesively compatible with said adhesive. 25

ALBIN H. WARTH.